

June 15, 1926.

1,588,617

N. A. ROSE

WATERPROOF OBJECT OR ARTICLE AND PROCESS OF PRODUCING THE SAME

Filed Sept. 1, 1923



Inventor:

*Newton A. Rose.*

By *Byrne, Townsend & Brickenstein,*  
Attorneys.

Patented June 15, 1926.

1,588,617

# UNITED STATES PATENT OFFICE.

NEWTON AUGUSTUS ROSE, OF WELLESLEY HILLS, MASSACHUSETTS.

## WATERPROOF OBJECT OR ARTICLE AND PROCESS OF PRODUCING THE SAME.

Application filed September 1, 1923. Serial No. 660,632.

This invention relates to waterproof objects or articles and particularly to tough resilient and waterproof wooden objects or articles.

An object of the invention is to provide a waterproof wood or article formed thereof which will have the toughness of wood with the resiliency of ivory. More specifically, an object of the invention is to provide a tough and resilient golf-club head which is unaffected by moisture.

According to my invention, I secure a resilient, tough and waterproof material by the impregnation of a wood of fine and substantially uniform texture with a synthetic resin. The only satisfactory woods of this type of which I am now aware are the woods of the genus *Nyssa*, commonly known as sour gum, cotton gum, etc. In these woods the fibrous structure or cells are remarkably uniform, with no marked difference in the size of the elements at the annual rings. These woods are also characterized by their freedom from parenchyma and ligno-cellulose and by the fineness of the tracheal elements and lack of the medullary rays which are characteristic of most exogenous plants. The substantially uniform and homogeneous composition of these woods with their utter lack of natural resin allows a ready and uniform impregnation with a fluid phenolic resin and when this is subsequently hardened by heat and pressure the resultant product is a mass of tough wood fibers which are reinforced and rendered waterproof and resilient by the phenolic resin: a product so different from the result obtained by the impregnation of other woods as to form a new material.

In forming a waterproof golf-club head, I prefer to shape the head and form the holes for receiving the shaft and weights before impregnating the wood. The holes assist in the ready impregnation of the wood, and small holes may be drilled in the head at other points, if desired, to facilitate the impregnation. After impregnation with a fluid phenolic resin, preferably by immersion and under pressure, such auxiliary holes may be closed with plugs formed of the same wood as the club-head before the phenolic resin is hardened by heat and pressure.

In the accompanying drawings:

Fig. 1 is a perspective view of a golf-club head; and

Fig. 2 is a vertical section on line 2—2 of Fig. 1.

In the drawings, the golf-club head which is indicated by the numeral 1 is formed of a wood having the very fine and substantially uniform texture which is found in the genus *Nyssa*. The head 1 is provided with an opening 2 for receiving the shaft and an opening 3 for receiving weights. If desired, additional holes 4 may be drilled into the head at points remote from openings 2 and 3 to provide for the ready introduction of the impregnating fluid into the wood. After the shaping and drilling of the club head 1, it is completely and uniformly saturated with a suitable phenolic resin by immersion under pressure. Following the saturation, the holes 4 of the head are filled with plugs 5, preferably of the same material as the head and similarly saturated, and the phenolic resin is hardened by heat and pressure according to known methods. When the phenolic resin has hardened the lead weight 6 may be cast in the opening 3 in the usual manner. Owing to the fact that the hardened phenolic resins are infusible at and above the melting point of lead, the molten lead may be cast in place without disturbing the uniformity of the impregnation.

Golf-club heads produced by my process are remarkably tough and resilient and cannot shrink or swell due to moisture absorption since the impregnation with a phenolic resin renders the head waterproof. When the wood is properly chosen, the resulting golf-club head is substantially homogeneous throughout and combines the qualities of the customary ivory inserts with the strength and toughness of the wood. It might be supposed that a satisfactory material for golf-club heads and for other articles which are subject to sudden shocks or strains could be produced by impregnating many of the natural woods with a phenolic resin. It is a remarkable fact, however, that the woods, which in their natural condition, possess properties which adapt them for such uses are found to lose some of these properties when rendered waterproof by impregnation with a phenolic resin. Although I have not made a thorough examination and comparison of the structures and properties of the woods which become brittle or inelastic when impregnated and the structures and properties of those woods which are tough and re-

silent when impregnated, it is my belief that the principal distinctions appear in the fine and even texture of the genus Nyssa and in their freedom from natural resin formations and from tannin.

While I have described the invention with reference to a golf-club head, it will be understood that other articles which must be tough, resilient and free from swelling or warping can be manufactured from impregnated woods of the genus Nyssa, and that the impregnating material may be a phenolic or other synthetic resin.

I claim:

1. A golf-club head comprising wood of

the genus Nyssa impregnated with a phenolic resin.

2. A golf-club head, the striking face of which comprises wood of the genus Nyssa impregnated with a phenolic resin.

20

3. A golf-club, the striking face of which comprises wood of the genus Nyssa impregnated with a synthetic resin.

4. A striking implement having an impact-receiving face comprising wood of the genus Nyssa impregnated with a phenolic resin.

25

In testimony whereof, I affix my signature.

NEWTON AUGUSTUS ROSE.